

## [54] LOAD BEARING CONCRETE PANEL RECONSTRUCTION

[75] Inventor: John H. Allen, Boulder, Colo.

[73] Assignee: Allen Research &amp; Development Corp., Boulder, Colo.

[21] Appl. No.: 299,618

[22] Filed: Jan. 23, 1989

## Related U.S. Application Data

[63] Continuation-in-part of Ser. No. 193,948, May 13, 1988, abandoned.

[51] Int. Cl.<sup>5</sup> E01C 7/00

[52] U.S. Cl. 14/73; 404/82; 14/1

[58] Field of Search 14/1, 17, 73; 404/70, 404/73, 82; 52/309.16, 309.17, 334, 602, 659, 743, 745; 428/247, 913; 264/31, 34, 35

## [56] References Cited

## U.S. PATENT DOCUMENTS

- 2,179,019 11/1939 Willetts 404/70 X  
 2,220,349 11/1940 Plumb 52/600 X  
 3,429,094 2/1969 Romualdi 52/659 X  
 3,808,085 4/1974 Givens, Jr. 52/659 X  
 4,565,840 1/1986 Kobayashi et al. 52/659 X

4,785,600 11/1988 Ting 52/334

Primary Examiner—Ramon S. Britts

Assistant Examiner—Matthew Smith

Attorney, Agent, or Firm—Donald W. Margolis

[57]

## ABSTRACT

Prior art supported, load bearing concrete panels having flexural reinforcing materials within the top and bottom halves, are over-designed, and experience increased deterioration and increased severity of cracks in the top surface due to flexural reinforcing materials which are located within the tip half of the panel. It is now taught that existing deteriorated concrete panels can be reconstructed by removing the upper concrete containing the upper layer of flexural reinforcing means for carrying bending moment tension stressed in the top half of panels (12), over interior supports (14), while maintaining such flexural reinforcing means (20) confined to the lower half of the panel, has sufficient flexural strength of the panel (12) to support expected loads. Such panels (12), will exhibit improved durability and reduced tip surface (16) cracking. Preferred techniques for controlling top half cracking from temperature and shrinkage of the panel are set forth.

18 Claims, 4 Drawing Sheets





FIG. I.  
PRIOR ART



FIG. 2.



FIG. 3.



FIG. 4.



FIG. 5.



FIG. 6.



FIG. 7b.

FIG. 7a.

PRIOR ART



FIG. 8.



FIG. 9.

## LOAD BEARING CONCRETE PANEL RECONSTRUCTION

### RELATED APPLICATIONS

This application is a continuation-in-part of U.S. patent application Ser. No. 193,948, entitled "Improved Concrete Panel Construction," filed by John H. Allen on May 13, 1988, abandoned.

### BACKGROUND OF THE INVENTION

#### (a.) Field of the Invention

The present invention relates generally to static structures. More specifically, it relates to concrete panel structures in a form which is useful for trusses or for use in bridge decks. The present invention also relates to methods of bridge construction and to methods of producing deck panels for use in bridge structures.

#### (b.) Description of the Prior Art

Typically, traffic bearing bridges are constructed using concrete bridge deck panels supported by a specifically designed substructure. Such concrete panels are normally supported at their longitudinal edges by at least a pair of separated support members, such as beams, which beams extend longitudinally in the same direction as what is defined herein as the length of the panels. State-of-the-art concrete bridge deck panel construction has traditionally been comprised of a slab constructed of one or more layers of concrete having a flexural reinforcing structure distributed throughout the concrete layer. Such a flexural reinforcing structure is generally in the form of a matrix of overlapping steel re-enforcing bars (re-bars) or steel strands, which are spaced from both the upper surface and the lower surface of the concrete panel. In accordance with traditional practice, this flexural reinforcing structure is included in the concrete for the purpose of carrying bending moment tension stresses which are placed on the concrete panel due to loading and unloading of the top surface, for example, by the passage of vehicles on or adjacent to the top surface.

It has traditionally been believed that structural flexural reinforcing material such as steel reinforcing bars (re-bars), are required throughout the concrete of such a panel, and especially in groups in the top and bottom halves of the panel near both the top and bottom surfaces of the panel. In the current state-of-the-art, it is believed to be necessary to use both top and bottom structural flexural reinforcing material re-bars in order to restrain cracking of the top surface and of the bottom surface due to applied loads.

The lower group of flexural reinforcing material in the bottom half of the panel normally consists of a first plurality of re-bars which form a layer. This first plurality of re-bars are transverse to both the length dimension of the panel and to the load-carrying beams which will support the panel. For structural purposes, this lower layer of transverse flexural re-bars material carries the positive moment tensile stresses which are applied to the panel. A second lower layer of flexural reinforcing material, consisting of a second plurality of re-bars which are parallel to both the length dimension of the panel and to the load-carrying, support beams (and transverse to the first lower layer of re-bars) is located directly above the first lower layer of re-bars. For structural purposes, this second lower layer of flexural reinforcing material re-bars distributes the bending moment loads which are applied to the panel

longitudinally. Both lower layers of flexural reinforcing material re-bars provide control of temperature shrinkage cracking at the lower surface of the panel. Under current codes, for most beam spacings which are up to about eleven feet apart, the longitudinal bottom group of flexural reinforcing material constitutes about one-half to about two-thirds of the main reinforcement of the panel. The two lower layers of flexural reinforcing material are usually joined together to form a mat or matrix.

Further, in accordance with current practice, another group of main flexural reinforcing material is located in the top half of the panel near the upper surface of the concrete panel. It consists of a first upper layer comprised of a plurality of flexural reinforcing materials, which are designed to carry the negative moment tensile stresses which are applied to the panel, and a second lower layer comprised of a plurality of flexural reinforcing materials, which are designed to hold the uppermost flexural reinforcing materials in position during concrete placement. Both upper layers of flexural reinforcing material re-bars are intended to provide control of temperature shrinkage cracking at the upper surface of the panel. The upper group of flexural reinforcing materials is also usually in the form of a mat or matrix, which matrix is sized and oriented substantially identically to and also parallel to the flexural reinforcing matrix group in the lower half of the panel.

The flexural reinforcing material composed of steel re-bars which are not coated or connected to a sacrificial anode corrode readily when exposed to thawing salts and other corrosive elements, and even to ordinary water.

Despite the above described traditional flexural reinforcing of concrete bridge deck panel structures, concrete bridge deck panels have been found to deteriorate rapidly and to require costly rehabilitation or replacement from time-to-time. It has been recently estimated, for example, that the use of thawing salts on bridges in the United States causes \$1.6 billion dollars worth of damage annually. Similar problems exist outside of the United States. Thus, there is a world-wide need to reduce the deterioration of concrete bridge deck panels without reducing the ability of the bridge deck panels to resist moment stresses imposed thereon by traffic loads.

It has been determined that much of the deterioration of concrete bridge deck panels is actually attributable to the corrosion of the traditional flexural reinforcing steel re-bars in the upper half of such bridge deck panels. It had been the common practice, until the late 1960's, to construct most concrete bridge deck panels over girder bridges with the bottom flexural reinforcing bars bent up over the supporting elements, such as beams or girders. Because of their shape, such bent up flexural strength reinforcing bars are sometimes referred to as "crank bars," because they resemble crankshafts. In the late 1960's the use of thawing salts on roads became quite prevalent. Subsequently the use of continuous straight flexural reinforcing top bars, or re-bars replaced the use of crank bars, because it was found to be more cost efficient to use more flexural reinforcing bars than to bend and place crank bars. As a result, this practice substantially increased the amount of corrodible steel re-bar material in the top of the deck panel. Bridge deck panels of this era were also constructed with only about 1.5 inches (3.8 cm) of protective con-

crete cover over the continuous straight top bars or re-bars.

During the early 1970's, the protective concrete cover over the top re-bars was generally increased to greater than about 2 inches (5.1 cm). At the same time, construction practices were improved so that reduction of the thickness of the top cover during panel placement, was avoided. It was believed that the additional thickness of the top cover would limit or slow cracking of the top surface, and thus lengthen the time that it took for chlorides from thawing salts and other corrosive elements to penetrate to the level of the re-bars contained in the upper portion of the concrete panel.

The understanding that chlorides from thawing salts and other corrosive materials corrode the re-bars in the upper half of the concrete panel and thus constitute the source of significant cracking and deterioration of the top surface of the bridge deck panel is important to the present invention.

Surprisingly, the additional thickness of concrete top cover included in bridge deck panel designs during the 1970's did not extend bridge deck panel life significantly. Subsequently, in most jurisdictions in which thawing salt is used, it became the practice to take steps to make bridge deck panels more impervious to the penetration of moisture, salt and other corrosive materials. It was believed that if the salt and other corrosive materials could not reach the re-bars in the upper half of the concrete layer, that the corrosion problem would be solved. Consequently, richer concrete mixes which were known to be more impervious to salts than traditional concrete mixes were utilized, and as a result the use of concrete having greater load bearing strengths then became standard practice. However, the use of richer concrete mixes led to yet another problem, in that such concrete exhibited increased temperature change shrinkage characteristics.

It is believed that the increased temperature shrinkage change of the richer concrete mixes may be responsible for additional cracks developing in the top surface of the concrete in recently constructed deck panel structures. Of course, such cracks will allow thawing salts and other corrosive materials to reach the corrodible re-bars in the upper half of the concrete panel and cause them to corrode, and thereby cause deterioration of the panel.

It is also known that cracking in the upper surface of concrete bridge deck panels can be avoided by careful control of the concrete mix and by concrete placement techniques. However, to be successful, such a strategy requires careful selection and proportioning of materials, and meticulous concrete placement and curing practice. These techniques have not been widely employed as part of a bridge deck construction strategy because it was thought that control of negative moment stresses in the upper surface of bridge decks was the dominate requirement for the restraint of cracking in the upper surface.

Several barrier technologies have been developed to stop or limit corrosion of flexural reinforcing re-bar materials which are located in the top half of concrete bridge deck panels from contact with thawing salts and other corrosive materials. Such barrier technologies include, for example, surface membranes, dense concrete, latex modified concrete, epoxy coated re-bars and the like. These barrier systems have had only moderate success.

Epoxy coated re-bars have proven to provide the most satisfactory corrosion protection, since such coatings, if continuous, virtually eliminate all actual contact between the re-bars and the thawing salts or other corrosive materials. However, it will be recalled that such re-bars are normally installed as matrices, which are often connected by tie wires and chains to the re-bar matrix in the lower portion of the concrete. The connecting tie wires and chains are usually electrically conductive. It has been found that placing a matrix of epoxy coated re-bars in the upper half of the concrete panel into electrical connection with the uncoated matrix of re-bars in the lower half of the panel allows an electrical half-cell to develop. The existence of such a half-cell encourages corrosion of the upper matrix of epoxy coated flexural reinforcing material. Additionally, epoxy coating re-bars apparently do not bond with the concrete in the panel as well as uncoated re-bars. Therefore, when epoxy coated re-bars are used in the top half of a concrete panel, once surface cracking is initiated, the length and width of cracks in the top surface tend to be larger than they would be had uncoated re-bar been used.

Waterproofing membrane barrier systems have been coated on the top surface of concrete panels. One potential problem with such waterproofing membrane barrier systems is that, should any moisture manage to migrate or collect below the membrane, it creates a severe environment in which corrosion can occur, whether or not salts or other corrosive materials are present. Furthermore, such barrier systems may conceal the deterioration of the top of the concrete from view, thereby delaying remedial maintenance until deterioration has become quite severe.

The above sequence of developments in the prior art of concrete bridge deck panels has been extremely costly. The combined effects of the additional thickness of the concrete, the use of epoxy coated re-bars in the upper portion of the bridge deck panel, the coating of waterproofing membrane systems on the top surface, and the increased girder weight necessary to carry the greater dead load of thicker deck panels, have all increased the cost of bridge deck panel systems by perhaps as much as 30-50%. Furthermore, despite the recognition of the problems caused by the corrosion of upper half flexural reinforcing re-bar, and the various technologies which have been developed to combat them, and even with the increased cost, deterioration of bridge deck panels still is a problem which has not been satisfactorily resolved.

Recently, a great deal of research has been conducted in an effort to develop means to protect the flexural reinforcing bar matrix in the top half of the panels from the effects of corrosion. The effectiveness of these efforts has been reported in National Cooperative Highway Research Program Report #297 (NCHRP 297), *Evaluation of Bridge Deck Protective Strategies*, September, 1987.

In the other known prior art, Mingolla U.S. Pat. No. 4,271,555 and Barnoff U.S. Pat. No. 4,604,841 are both examples of bridge deck panel structures which attempt to overcome certain problems of construction. However, while there are certain novel features to these particular deck panel constructions, both of them use conventional flexural reinforcing steel bar materials near both the upper as well as the lower surface of the deck panel structure.

Recent known patents which have been awarded for bridge deck protection systems, include Jacobs U.S. Pat. No. 4,151,025; U.S. Pat. No. 4,708,888; and Marzocchi U.S. Pat. No. 4,319,854. They teach, respectively, a membrane barrier system, an electro-chemical "cathodic protection" system, and a combination membrane and electro-chemical system.

Through various research efforts, it has been found that transverse cracking generally occurs at the top surface of the panel substantially directly over the layer of transverse flexural reinforcing bars which are in the top half of a bridge deck panel. Such cracks are a significant factor in the deterioration of bridge deck panels, since, as already noted, they allow salts, other corrosive elements, and water to reach the flexural reinforcing bars which are in the top half of the panel and cause them to corrode, thereby accelerating deterioration of the panel. Surprisingly, these cracks form at about right angles to the direction that they would be expected to form if they were due to the stresses caused by the predicted bending moments to which the panel is subjected. However, it is now noted that the observed crack patterns are consistent with tensile stresses due to concrete shrinkage and the effects of temperature changes. This indicates that the control of the formation of transverse cracks directly over the top transverse reinforcing bars due to concrete shrinkage and temperature changes at the surface of bridge deck panels is of paramount importance in avoiding deck panel deterioration. However, effective means for its avoidance are not known to have been previously proposed.

It is well known that the use of either fibers or fabric serves to effectively control upper surface cracking due to volume changes from temperature and shrinkage. Such reinforcement materials can be used, in at least the concrete which forms the uppermost portion of a bridge deck panel, to control surface cracking caused by temperature shrinkage changes does not require careful control of the concrete mix, nor careful placement of the concrete in order to be successful. Romauldi U.S. Pat. No. 3,429,094 and Kobayashi U.S. Pat. No. 4,565,840 teach the use of fiber reinforcement materials for crack control in concrete. The use of various fiber materials for reinforcement concrete is discussed in the *Manual of Concrete Practice*, ACI. The use of fiber reinforcement materials to restrain cracking due to changes from temperature shrinkage has now become more common than the well established practice of using steel welded wire fabric reinforcement materials for such purposes, see Romauldi U.S. Pat. No. 3,429,094.

Also noted as of interest are Graham U.S. Pat. Nos. 865,490 and 983,274; Henderson U.S. Pat. No. 1,891,763; Rubenstein U.S. Pat. No. 2,850,890; Naaman U.S. Pat. No. 3,852,930; Schupack U.S. Pat. No. 4,159,361; and Matsumoto U.S. Pat. No. 4,379,870; as well as U.K. Patent No. 578,036; Japanese Patent No. 2,141,206; and German Patent No. 3,342,626. Of these, Graham U.S. Pat. Nos. 865,490 and 983,274 disclose a reinforced concrete slab which is designed and intended for placement on the ground. These references includes reinforcing rods in the bottom half, with the latter of these references including the addition of what appears to be a high volume of short wire sections in the upper portion of the concrete to increase the strength of the slab. Because of the size and volume of the wire sections they are added by placing them on top of the concrete and allowing them to settle into the concrete. Graham neither teaches nor suggests a load bearing panel in-

tended to be placed on two or more spaced apart supports, and in the more than eighty years since its filing, its application to load bearing panel construction technology is not known to have occurred. Schupack U.S. Pat. No. 4,159,361 discloses cold formable, reinforced panel structures which include shrinkage and thermal reinforcement fibers. Schupack neither teaches nor suggests a load bearing panel which is intended to be placed on two or more spaced apart supports, nor a panel which includes flexural reinforcing material, and its application to load bearing panel construction technology is neither taught nor suggested. Matsumoto U.S. Pat. No. 4,379,870 discloses a specific form of synthetic resin reinforcement material which has utility in concrete structures, but it neither teaches nor suggests a load bearing panel which is intended to be placed on two or more spaced apart supports, nor a panel which includes flexural reinforcing material, and its application to load bearing panel construction technology is neither taught or suggested.

It is important to here note that "reinforcement material" as used throughout this application is different from "flexural reinforcing material," such as traditional steel re-bars.

#### SUMMARY OF THE INVENTION

Accordingly, it is a principal object of the present invention to provide a load bearing concrete panel which is significantly less expensive than existing panels due to the removal of materials which are now used in state-of-the-art load bearing concrete panels without loss of the utility of such panels, and, in fact, with improved durability of the resulting panels.

A further object of the present invention is to provide a method of making load bearing concrete panel which requires less steps and which is significantly less expensive than existing panels due to the elimination of steps which are now used in the state-of-the-art process for producing load bearing concrete panels without loss of the utility of such panels, and, in fact, with improved durability of the resulting panels.

Yet another object of the present invention is to provide a concrete bridge deck panel structure which has sufficient flexural reinforcement to provide the appropriate amount of flexural strength, while also being designed to eliminate or at least significantly impede the amount and speed of surface deterioration of the deck panel.

Still yet another object of the present invention is to provide a concrete bridge deck panel structure in which structural flexural reinforcing material, such as steel reinforcing bars, are not required in the top half of the panel near the top surface of the panel.

Another object of the present invention is to provide a concrete bridge deck panel structure in which structural flexural reinforcing material composed of steel need not be epoxy coated or connected to a sacrificial anode in order to prevent corrosion of such flexural reinforcing material which will cause deterioration of the top surface of such a panel.

It is yet another object of the present invention is to provide a concrete bridge deck panel structure in which chlorides from thawing salts and other corrosive materials do not corrode re-bars in the upper half of the concrete panel with the avoidance of a source of significant cracking and deterioration of the top surface of the bridge deck panel.

Yet a further object of the present invention is to provide a concrete bridge deck panel structure in which increased temperature and volume change shrinkage due to the use of richer concrete mixes is avoided in the top surface of the concrete.

Still yet another object of the present invention is to provide a crack and corrosion resistant concrete bridge deck panel without reducing the ability of the bridge deck panel to resist moment stresses imposed thereon by traffic loads.

Another object of the present invention is to provide a bridge deck panel which resists cracking at the upper surface of the panel due to concrete volume shrinkage and temperature changes.

A further object of the present invention is to provide a load bearing concrete panel structure having improved structural properties which prevent or reduce deterioration of the top surface of the panel caused by corrosion of flexural reinforcing materials.

It is a further object of the present invention to provide a load bearing concrete panel structure having improved structural properties which eliminate the cracking or deterioration of the top surface of the panel caused by corrosion stress from transverse flexural reinforcing materials.

Still yet another object of the present invention to provide a concrete bridge deck panel structure having improved structural properties which prevent or reduce deterioration of the top surface of the panel due to temperature and shrinkage volume changes at the top surface.

Another object of the present invention is to provide a concrete panel for use in new bridge construction as well as a process for producing such concrete panels and also for use in rehabilitating existing panel structures, which panel design reduces the corrosion characteristics of the top half and top surface of the panel.

Yet another object of the present invention is to provide a concrete panel design for use in new bridge construction and in rehabilitating existing bridge panel structures, which panel design inhibits deterioration of the top surface of the panel due to temperature and shrinkage volume changes at the top surface.

As discussed in detail above, substantially all known efforts previous hereto to reduce the problem of the corrosion of flexural reinforcing materials have been defensive in nature. That is they have either sought to isolate top flexural reinforcing material from corrosive compositions, for example by the provision of a greater amount of concrete top cover or a water proof membrane on the concrete above the top flexural reinforcing re-bars, or by epoxy coating the re-bars, or they have used electro-chemical methods, such as cathodic protection. However, these solutions do not deal with or solve what is now recognized by the present invention to be a two-fold problem with existing bridge deck panel designs. It is now recognized that problems of panel deterioration and top surface cracking are caused by the flexural reinforcing materials, such as corrodible re-bars, which are located within the top half of the concrete panel, and especially such flexural reinforcing materials which are near the top surface of the panel and oriented transversely. This is due to the fact that the flexural reinforcing materials which are in the top surface of the panel are subject to corrosion and accelerate degradation of the surface of the panel, and those which are near the top surface of the panel and oriented transversely have now been determined to accelerate the

widening and increase the severity of cracks in the top surface due to temperature shrinkage changes.

Having recognized the above enumerated problems, the present invention suggests new solutions which are quite different from the defensive solutions utilized in prior and current deck panel designs. It is now postulated that the current practice of placing corrodible flexural reinforcing materials, such as steel re-bars, in the upper half of a concrete bridge deck panel, and especially transversely oriented flexural reinforcing materials which are near the top surface of the panel, is far more detrimental than beneficial to the long term performance of the panel. Therefore, the use of flexural reinforcing materials, and especially of steel reinforcing bars, in the top half of a bridge deck panel, as currently practiced, adversely affects the durability of the panel.

Elaborating, this postulate is based on the facts that: (1) transversely oriented flexural reinforcing materials, such as reinforcing bars, apparently contribute to increased transverse crack formation due to temperature induced concrete shrinkage at the surface of the panel; (2) when corrodible flexural reinforcing materials in the upper half of a bridge deck panel are exposed to corrosion causing materials and solutions, they corrode and thereby accelerate the deterioration of the surface and the top half of the panel; (3) flexural reinforcing materials, are not required in the top half of a panel for structural strength of the panel; and (4) under standard practices, adequate amounts and distributions of flexural reinforcing materials are present in the bottom half of the panel to provide sufficient flexural strength to the panel.

It has therefore now been discovered, in accordance with the present invention, that the placement of transverse reinforcing bars in the upper portion of bridge deck panels is not required to provide adequate structural strength to such panels, and that the top layer of longitudinal re-bar is not effective in controlling cracking of the upper surface. It has further been discovered, in accordance with the present invention, that the placement of any flexural reinforcing materials in the upper half of bridge deck panels is not required to provide adequate structural strength to such panels. It is further postulated that various crack control practices at the upper surface of deck panels, other than the state-of-the-art use of flexural reinforcing material, should be the governing design criterion for crack control at the top surface of the upper half of bridge deck panels, and that flexural reinforcing means should be confined to the lower portion of the bridge deck panel.

Crack control of the upper surface of deck panels can be improved using several practices. First, and most preferably, concrete mix compositions can be used which resist surface cracking associated with changes due to temperature shrinkage design properties, and such concrete compositions should be the subject of careful placement practice and curing. A second manner of improving crack control at the upper surface of a deck is by the use of fibrous reinforcement materials, preferably in the upper quarter to one-half of the panel. A third manner of improving crack control at the upper surface of a deck is by the use of a reinforcement fabric in the uppermost region of the panel in order to resist shrinkage changes due to temperature. A small volume of steel welded wire fabric is typically used for this purpose. For best crack control reinforcement, in accordance with the present invention, fiber or fabric reinforcement materials should be placed as close to the

upper surface as practicable, preferably no lower than about one-sixth of the total depth of the concrete panel. For bridge deck panels of 7½ to 9 inches thick, this is typically less than 1½ inches from the surface.

Since it has been determined by the present invention that bridge structures, as they are presently being designed, are in fact being over-designed by the inclusion of flexural reinforcing material; and since it has been further determined that top flexural reinforcing material placement, in accordance with current practice, adversely affects corrosion resistance and crack formation; it has therefore now been discovered that the flexural reinforcing material in the top half of existing bridge deck panel structures can be entirely removed without reducing the strength of the panels below what is sufficient to meet the demands which they must meet. It has been determined that with flexural reinforcing material in only the lower half of a bridge deck panel, more than sufficient flexural strength for moment bending stresses of the panel will be provided. It will be readily appreciated that the removal of two layers of flexural reinforcing material from the panel that there will result in substantial reductions in production steps and in the cost of materials and the costs of construction.

It is therefore now taught that bridge deck panels with a flexural reinforcing material re-bar matrix in only the lower half of the panel, in accordance with the practice of the present invention, and preferably substantially no reinforcement material, in the upper half of the bridge deck panel have substantially improved durability. A bridge deck panel with the top portion of the deck panel constructed in accordance with the current teaching does not require an extra thickness of concrete cover, or other of the expensive prior art defensive measures, thus, simultaneously, achieving both great cost savings and improved panel durability.

Therefore, to achieve the foregoing and other objects, and in accordance with the purposes of the present invention, a new and improved concrete panel design for use as a bridge deck panel in a bridge structure, or the like is disclosed. The panel design includes at least one layer of concrete which has flexural reinforcing material disposed only within about the lower half, and preferably in the lower one-third to about one-sixth of the concrete panel. The flexural reinforcing material may be even lower if the applicable codes will allow it. In preferred embodiments, a minimum of reinforcement material, such as fiber or fabric may be disposed in the panel, preferably in about the upper one-third to one-half portion of the concrete layer to provide control of cracking due to temperature shrinkage.

In an alternative embodiment, a small amount of widely spaced flexural reinforcing re-bars, preferably oriented in the longitudinal direction, may be used in the upper half of a panel to reduce surface cracking.

These and other objects of the present invention will become apparent to those skilled in the art from the following detailed description, showing the contemplated novel construction, combination, and elements as herein described, and more particularly defined by the appended claims, it being understood that changes in the precise embodiments of the herein disclosed invention are meant to be included as coming within the scope of the claims, except insofar as they may be precluded by the prior art.

#### BRIEF DESCRIPTION OF THE DRAWINGS

The accompanying drawings illustrate complete preferred embodiments of the present invention according to the best modes presently devised for the practical application of the principles thereof, and in which:

5 FIG. 1 is a front perspective schematic cut-away view, partially in phantom, of a typical prior art bridge deck panel supported on girders, showing the structure 10 of the deck panel with flexural reinforcing material in both the upper and the lower half of the panel;

10 FIG. 2 is a front perspective schematic cut-away view, partially in phantom, of one embodiment of a bridge deck panel according to the present invention, supported on girders, showing the structure of the deck panel with flexural reinforcing material in only the lower half of the panel;

15 FIG. 3 is a cross-sectional schematic view of a deck panel of the present invention which is similar to the panel shown in FIG. 2;

20 FIG. 4 is a cross-sectional schematic view similar to FIG. 3 and illustrating a second embodiment of the present invention, including fiberous reinforcement material in the concrete;

25 FIG. 5 is a cross-sectional schematic view similar to FIGS. 3 and 4 and illustrating yet a third embodiment of the present invention, including woven wire reinforcement material in the concrete;

30 FIG. 6 is a cross-sectional schematic view similar to FIGS. 3, 4 and 5 and illustrating an embodiment of the invention which is useful with pre-cast panel structures;

35 FIG. 7A is an enlarged cross-sectional schematic view of a typical prior art bridge deck panel, similar to the panel shown in FIG. 1, positioned for comparison with FIG. 7B;

40 FIG. 7B is an enlarged cross-sectional schematic view of a deck panel structure, including fiberous reinforcement material in the upper half of the concrete, similar to FIG. 4 of the present invention, as utilized for refurbishing existing bridge panel structures;

45 FIG. 8 is an enlarged cross-sectional schematic view similar to FIG. 3 illustrating yet another embodiment of the present invention; and

45 FIG. 9 is a longitudinal schematic view, partially in cross-section of a bridge deck panel structure illustrating an embodiment of the present invention which is useful in portions of the concrete bridge deck panel which are in the vicinity of a support, in which the bridge superstructure is continuous over such a support.

#### DETAILED DESCRIPTION OF THE DRAWINGS

Referring first to FIG. 1, a portion of a state-of-the-art bridge structure, generally 10, is illustrated in a front perspective schematic cut-away view, partially in phantom. Bridge structure 10 includes a concrete bridge deck panel 12 supported by beams 14. Bridge deck panel 12 includes a top surface 16 and a bottom surface 24. An optional waterproofing membrane 17 is shown as overlying top surface 16 of panel 12. Waterproofing membrane 17 is used to protect bridge deck panel 12 from the intrusion of corrosive solutions. Waterproofing membrane 17 is then overlain by wearing course 18 which is intended to come into contact with loads, such as vehicle traffic, which traverse panel 12 and bridge structure 10. For purposes of discussion, panel 12 may be considered as having a concrete layer 22 separated into an upper half 28 and a lower half 29 by a plane 32.

In this prior art bridge structure 10, two groups of flexural reinforcing materials, in this case in the form of matrices of steel reinforcing bars, are located in concrete panel 12, one in the upper half and one in lower half 29 22. Lower group 20 of flexural reinforcing materials is below plane 32, closely adjacent to bottom surface 24 in lower concrete half 29. Lower group 20 of flexural reinforcing materials includes a lower layer of flexural reinforcing bars 21 which are oriented transverse to the longitudinal direction of panel 12, and an upper layer of longitudinal flexural reinforcing bars 23 which are oriented longitudinally, that is in the same direction as the longitudinal direction of panel 12. Layer 21 of flexural reinforcing bars are provided to resist positive transverse flexural moments which are applied to panel 12. Layer 23 of flexural reinforcing bars are provided to resist longitudinal positive flexural moments which are applied to panel 12. This lower group 20 of flexural reinforcing materials 21 and 23 also acts to control temperature and shrinkage crack formation in bottom surface 24. Flexural reinforcing bars 21 and 23 form bottom reinforcing mat 20.

An upper group 30 of flexural reinforcing materials is above plane 32, closely adjacent to upper surface 16 in upper concrete half 28. Upper group 30 of flexural reinforcing materials includes an upper layer of flexural reinforcing bars 35 which are oriented transverse to the longitudinal direction of panel 12, and a lower layer of longitudinal flexural reinforcing bars 37 which are oriented longitudinally, that is in the same direction as the longitudinal direction of panel 12. Layer 35 of flexural reinforcing bars are provided to resist positive transverse flexural moments which are applied to panel 12. Layer 37 of reinforcing bars are provided to control temperature and shrinkage cracking in upper surface 16, and to maintain alignment of bars 35 during concrete placement. Flexural reinforcing bars 35 and 37 form a top reinforcing mat 30 in the upper half of panel 12 which in fact, normally provides more flexural strength to panel 12 than is necessary for the intended use of the panel.

For the purposes of this particular specification, the following terms are defined as follows:

1. "Longitudinal" is the direction of support beams 14 and of the normal flow of traffic along upper surface 16;
2. "Transverse" is the direction, along surface 16, which is at right angles to the longitudinal direction and also at right angles to support beams 14;
3. "Positive moment" (+M) causes tension on lower surface 24 of concrete panel 12; and
4. "Negative moment" (-M) causes tension in upper surface 16 of panel 12.

As set forth above, and as now applied to FIG. 1, observations of current bridge structure, construction and degradation, disclose that longitudinal cracking and de-lamination over girders 14 is no more severe than longitudinal cracking and de-lamination at other areas of deck panel 12. It has also been observed that cracking in negative moment regions at the top of continuous spans is no more severe than cracking which occurs elsewhere. It has also been discovered that transverse cracks in upper surface 16 of deck panel 12 are more prevalent than longitudinal cracks. The conclusion that can be reached from these observations and discoveries is that longitudinal tensile stresses due to continuity, dynamic effects and concrete shrinkage are more significant as a cause of transverse cracks in upper surface 16 of deck panel 12 than are transverse stresses. Similarly,

the conclusion can be reached that transverse stresses cause longitudinal cracks. However, current bridge deck panels, such as those illustrated in FIG. 1, are reinforced with both top and bottom flexural reinforcing materials oriented in the transverse direction of the panels. Consequently, this results in increased transverse cracking in upper surface 16 of deck panel 12 due to longitudinal stresses, with crack formation often occurring directly over upper transverse flexural reinforcing members 35. Such crack formation over upper transverse flexural reinforcing members 35 subsequently provides a path by which layer 30, comprised of flexural reinforcing members 35 and 37 are exposed to thawing salt and other corrosion causing compositions which cause accelerated corrosion of those flexural reinforcing members, and as a result more deterioration of the panel and cracking of upper surface 16. Therefore, the formation of transverse cracks directly over upper transverse flexural reinforcing bar members 35 is now seen to be a major problem in bridge deck panel deterioration.

Referring next to FIG. 2, there is illustrated a front perspective schematic cut-away view, partially in phantom, of one embodiment of a bridge deck panel 12 according to the present invention, bridge structure 10. In FIG. 2 like numbers refer to the same elements as in FIG. 1. Bridge structure 10 includes a concrete bridge deck panel 12 supported by a plurality of spaced-apart, longitudinally aligned beam supports 14. Support beams 14 may be steel girders, webs of box girders, concrete girders or any other art known means to support a concrete deck panel structure. For purposes of discussion, panel 12 may be considered as being separated into an upper half and a lower half 29, as in FIG. 1. Support beams 14 are in turn transversely supported by art known bridge foundations (not illustrated), such as bents, piers and abutments. In normal usage, parapets (not illustrated) will be positioned along each of the longitudinal edges of bridge deck panel 12 to define a passageway for cars, trucks, and other traffic, as well as for pedestrians across or closely adjacent to upper surface 16. It should be noted; however, that bridge deck panel 12, as illustrated in FIG. 2, includes a matrix group of flexural reinforcing bar materials 20 embedded only in the lower half 29 of the panel juxtaposed to bottom surface 24 of deck panel 12, but that it includes no flexural reinforcing bar materials in the upper half of panel 12.

Referring more specifically to the preferred embodiment of the invention which is disclosed in FIG. 2, it will be noted that it completely eliminates steel flexural reinforcing bars from the top half of panel 12. So, for example, given a panel having a thickness of about eight inches (20.3 cm) about four inches (10.2 cm), or the upper half 28 of the bridge deck panel 12, whichever is greater, includes no steel flexural reinforcing bars. This is in sharp contrast to the current practice, illustrated in FIG. 2, of placing large flexural reinforcing bars in the top half of a given panel 12 also having a thickness of about eight about inches (20.3 cm), in the upper half about two inches (5.1 cm) or more below top surface 16, which practice has in fact been found to significantly increase the severity of cracking and concrete shrinkage cracking at top surface 16. Thus, as discussed above, while the use of flexural reinforcing bars in the upper half of a panel normally provides more flexural strength to panel 12 than is necessary for the intended use of the panel, the presence of flexural reinforcing bars in the

upper half aggravates the problem of cracking due to temperature changes and concrete shrinkage due to underlying corrosion, with the result that cracking and deterioration of the panel is accelerated by the presence of flexural reinforcing bars in the upper half of the panel. Therefore, in accordance with the present invention, as shown in FIG. 1, a concrete layer 22 is provided which includes standard flexural reinforcing materials, for example primary steel flexural reinforcing grid 20 or other flexural strength reinforcing material in the bottom half of bridge deck panel 12, with no flexural strength reinforcing material in the top half of panel 12, either between or over supporting members 14. In the most preferred embodiment, the upper mat 30 of flexural reinforcing material is eliminated from the upper portion of the deck panel and the structure relies substantially solely upon the concrete itself for thermal and shrinkage crack resistance.

Once the flexural strength reinforcing material has been excluded from the top half 28 of panel 12, in order to best control cracking at the top surface 16 due to concrete shrinkage, the concrete deck panel 12 should be constructed, at least at the upper half 28, employing: either a concrete formulation having concrete shrinkage volume change compensating properties and adequate tensile strength to resist stresses from temperature change and concrete shrinkage change; or fibrous reinforcement material uniformly distributed throughout top portion of deck panel; or reinforcement material for temperature and shrinkage reinforcement material such as closely spaced small diameter wires or small diameter wire fabric.

Referring now to FIG. 3, there is shown a cross-sectional schematic view of deck panel 12, which is similar to the panel shown in FIG. 2. As illustrated it includes a concrete layer 44 having standard re-bar flexural reinforcing material 20 along the bottom portion thereof. In this particular embodiment the concrete composition of at least the upper half of concrete layer 44 is formulated to resist cracking from concrete shrinkage due to temperature change. The concrete in panel 12 of this example may be placed in one or more layers. Crack formation due to concrete shrinkage from temperature change can also be controlled and minimized by other known methods of controlling the concrete composition, including the selection of size and type of coarse aggregate, water-cement ratio, cement-aggregate ratio, cement type, concrete placing sequence, and cement curing methods. Therefore, the key to the embodiment of FIG. 3 is to increase the tensile strength of the concrete mix for layer 44 to higher than normal, and to select concrete mix formulation or placement practice or curing practice that minimize shrinkage changes.

Referring now to another preferred embodiment as illustrated in FIG. 4, a typical cross section of a bridge deck panel 12 is illustrated showing a layer of concrete 22 having a matrix of standard bottom deck panel flexural reinforcing re-bar 20 in the lower half 29 thereof. FIG. 4 further illustrates an embodiment of the present invention wherein the concrete includes a fibrous reinforcement material 34 uniformly distributed throughout. In other embodiments the concrete may include fibrous reinforcement material distributed throughout only the upper half, and preferably in only the upper 40% as indicated by line 32.

The fibrous reinforcement materials are preferably made from steel, polymeric materials, such as polypropylene, or other material suitable for use in a high alka-

line and salt saturated environment. The volume of fiber which is used should be sufficient to increase the cracking modulus of the concrete matrix up to about 750 psi. The percentage of fiber reinforcement required to provide that amount of effective crack control will depend upon the physical and geometric properties of the fibers. For structures exposed to de-icing chemicals, ACI (American Concrete Institute) recommends the flexural crack width not be allowed to exceed 0.007 inch (0.018 cm). The limiting width for temperature and shrinkage cracks might appropriately be less than this, but certainly should not exceed the allowable crack width for structures exposed to weather, which is 0.012 inch (0.03 cm). Therefore in the practice of the present invention it is recommended that the temperature volume change crack control reinforcement limit crack width to the range of about least 0.005 inch (0.013 cm) to about 0.01 inch (0.025). This may usually be accomplished by using fibrous reinforcement material of from about 0.5% to about 4%, by volume, within the top one-half of deck panel 12. For example, the percent volume of steel fiber reinforcement is usually preferably less than 1%, but may be as much as 2% or greater. Fibrous reinforcement materials such as steel fibers coated with polymer, or stainless steel or polymeric materials are desirable because they avoid corrosion. These, and other non-corrodible fiber reinforcement materials for concrete, are commercially available. The art of fiber reinforced concrete is well known and described in the section 30 "Fiber Reinforced Concrete", *Manual of Concrete Practice*, ACI.

Referring to FIG. 5, deck panel 12 is illustrated supported on beams 14 and includes a concrete layer 22 having standard bottom flexural reinforcing bars 20 as discussed previously. FIG. 5 further illustrates another embodiment of the present invention wherein reinforcement material for temperature shrinkage crack control purposes is provided in the upper portion of concrete layer 22. In this instance the reinforcement material is a welded wire fabric 38. Wire fabric 38 is comprised of longitudinally arranged wires 40 and transversely arranged wires 42. In this preferred embodiment wires 40, 42 would normally be less than about 0.3 inch (0.76 cm) in diameter, and are preferably equally spaced in both the longitudinal and transverse directions so as to control the temperature change cracking and concrete shrinkage cracking at upper surface 16. The cross sectional area of the fabric should conform to the current code recommendations for temperature and shrinkage reinforcement, that is 0.11 square inch per foot width in each direction. Wire spacing should not exceed the thickness of panel or overlay. In one preferred form, wire spacing may vary between about two and about six inches (5.1 and 15.3 cm). To control placement of welded wire fabric in the top one inch of concrete, which is the most preferred embodiment, wire fabric should be pressed into concrete from the surface thereof. The fabric 38 should be placed no closer to surface 16 than three times the diameter of individual wires 40 and 42, which will normally be between about  $\frac{1}{4}$  inch and one inch from top surface 16 of deck panel 12. If steel wires of different diameters are provided in each direction, the ratio of the areas should be approximately proportional to the ratio of the length to width 60 of the panel, with the larger cross-sectional area per unit width wire running in the longer dimension.

Web 38 may be composed of synthetic fabric in lieu of a steel fabric as discussed above, but the tensile force

capacity per unit width should provide at least that of the type of steel fabric previously specified. The maximum cross-sectional area of the synthetic fabric used should be at least in proportion to the ratio of Young's modulus of the synthetic material to Young's modulus of steel. The equivalent cross-sectional areas, texture, openings and the distance from the surface and spacing requirements as specified for a steel fabric should also be met by such a synthetic fabric. Further, the synthetic fabric should provide the same recommended temperature and shrinkage crack control as are required of reinforcement fibers, and described above.

Panel placement as illustrated in FIGS. 3, 4 and 5, may be continuous and monolithic, or it may be placed in discontinuous sections, separated by vertical bulkheads to control concrete shrinkage strains. Panel placement may also be in discontinuous vertical lifts to reduce the quantity and cost of temperature change and concrete shrinkage crack resistant concrete used. Proper curing and bonding at the interface between placements must also be maintained.

Referring now to FIG. 6, there is illustrated a structure showing how the present invention may be utilized in conjunction with pre-cast concrete deck panel systems. In this embodiment, of deck panel 12, pre-cast lower or bottom concrete panels 50 are shown supported on and between girders 14. Pre-cast panels 50 include flexural reinforcing members 20 incorporated therein. Once pre-cast panels 50 are placed and interconnected into position on girders 14, a continuous cast-in-place concrete topping 52 comprised of either plain concrete or including fibrous reinforcement or welded wire fabric, as described above, may then be positioned over pre-cast panels 50. In this manner, pre-cast panels 50 can be constructed in accordance with required flexural strength requirements of the particular bridge system being designed, and concrete top layer 52 may be placed over the pre-cast concrete without having to provide additional flexural reinforcing material, other than for concrete shrinkage or thermal crack control purposes.

Referring to FIG. 7B, the present invention may also be utilized in refurbishment of existing bridge deck panels. In this instance, bottom portion 54 of bridge deck panel 12, including its original flexural reinforcing members 20, is retained in place, while the prior upper layer 56 and upper mat of flexural reinforcing 30, as shown in FIG. 7A, are removed. In this case it is assumed that the upper layer of concrete 56 was chloride contaminated and the upper mat 30 of flexural reinforcing material was corroded and causing cracking, spalling and delamination of bridge deck panel 12, thus establishing the need to remove concrete 56 and upper re-bar mat 30 and refurbish deck panel 12. In the preferred practice of the present invention, not only are the upper portions of concrete 56 removed, but so are any portions of bottom portion 54 which are found to have a chloride content greater than about 0.1% by volume. Remaining bottom portion 54 includes existing re-bar flexural reinforcing structure 20. A continuous cast-in-place concrete topping 57 is then be placed over remaining layer 54, with anchor bolts 58 being provided as required to assist the bonding of new concrete layer 57 to original layer 54. As can be seen in FIG. 7B, fiber reinforcement material 59 is dispersed throughout new upper layer 57 in accordance with the teaching of the present invention, as described above. Moreover, welded wire fabric or specially formulated concrete

may also be utilized in layer 57 in accordance with the details set forth above.

The side-by-side comparison of FIGS. 7A and 7B are also useful in contrasting the difference in the basic structure of the prior art panel and the panel of the present invention. In the prior art panel 12, as shown in FIG. 7A, the flexural reinforcing members 30 are present in upper half 28. In the present invention, as represented by FIG. 7B, there are no flexural reinforcing members in the upper half of panel 12, and yet the utility of such panels is not lost, and which, in fact, exhibit improved durability and resistance to deterioration.

Referring to FIG. 8, the present invention may also be utilized with a structural steel deck panel 60, which is commonly known as a "stay-in-place" form. In this embodiment structural steel deck panel 60 is used in conjunction with standard lower half flexural reinforcing re-bar matrix 20. Once structural steel deck panel 60 is laid in place in conjunction with flexural reinforcing 20, concrete, for example, including fiber reinforcement 62 is then laid over deck panel 60 and flexural reinforcing re-bar matrix 20. The steel deck panel 60 may be constructed and positioned in accordance with known bridge construction techniques.

Finally, FIG. 9 illustrates an embodiment of the invention wherein the panels are utilized in the construction of a continuous bridge. In this instance, lower half 64 of deck panel 12 includes a lower matrix of standard flexural reinforcing re-bars 20 as previously discussed. Upper layer 66 is shown to include wire web 68 which is utilized as reinforcement to restrain cracking of upper surface 16 from concrete shrinkage due to thermal changes. Upper layer 66 is also shown as including additional longitudinal flexural reinforcing bars 70 in the upper portion of panel 12 overlying support beam 14. Top longitudinal flexural bars 70 are placed to provide additional reinforcement to restrain cracking in the deck from bending moments in the bridge. However, it is important to the present invention to note that there are no transverse flexural reinforcing bars located in upper half 66. Flexural reinforcing bars 70 should be approximately 2 inches or more below top surface 16, as in present bridge construction practice. Top longitudinal flexural bars 70 are placed to restrain cracking in the deck from bending moments in the bridge. Because the rate of change of stress in concrete is dependent on the total depth of the panel plus girder, effective crack control will normally be obtained when flexural reinforcing bar 70 is placed no further from top surface than about 5% to about 10% of the total depth of the panel and supporting girders or beams 14. As with the practice described above, this embodiment may also include special concrete formulations and practice, fiber reinforced concrete or fabric embedded in the upper half of the concrete. The present invention also simplifies the process of constructing bridge deck panels. State-of-the-art bridge deck panel construction processes, utilizing traditional techniques, are formed in place on primary girders which provide longitudinal support. A bridge deck panel is constructed using the steps of installing either permanent or removable forming and falsework for shoring and bracing necessary to support the concrete bridge deck panel, shown generally as 80 in FIG. 4. Next, chairs or supports for the lower flexural reinforcing matrix are positioned. Next, the lower flexural reinforcing matrix is placed upon chairs and tied together in accordance with standard construction and detailing practices. Then, supports for the upper

flexural reinforcing matrix are positioned. These supports are known as "high chairs". After the chairs which support the upper flexural reinforcing matrix are placed, then an upper flexural reinforcing matrix is installed. Then concrete material is placed in the forms, finished, and cured, thereby providing a structural bridge deck panel. Finally, an optional concrete overlay or membrane system, for example with a bituminous wearing surface, is installed. Falsework and removable portions of the forming are removed after the concrete has obtained sufficient strength.

An alternative to this traditional method of making concrete bridge deck panels on multi-beam bridge superstructures, is to first place pre-fabricated deck panels between and/or over supporting beams. Then soffit forms and soffit reinforcing are installed as required, followed by the installation of supports for an upper flexural reinforcing matrix. The upper flexural reinforcing re-bar matrix is then installed, the concrete material is placed, and then cured and finished as previously described.

The improved process to which this invention applies considerably reduces both the number of steps and the amount of materials necessary to construct a concrete panel which is suitable for supporting superimposed loads. The improved process of panel construction, according to the present invention, is applicable to both panels which are fully cast in place, as well as to panel which is cast to include pre-existing pre-cast concrete, which is cast to include pre-existing steel bridge deck material, and to the refurbishment of existing panels.

The process is applied to the construction of panels which are fully cast in place, in that the steps of placing primary longitudinal beams for bridge superstructure and of placing are forming and falsework, shoring, and bracing is the same as in the basic traditional process described above. The reinforcing chairs for the lower mat are also placed, as is the lower reinforcing bar mat as described in the basic process. The step of placing reinforcing chairs for the upper mat and the placement of the upper reinforcing bar mat, as described in the basic process, are eliminated, as are the materials for those chairs and mats. The concrete is then placed, finished and cured, as described in the previous process. The last step of removing falsework is then completed.

In the preferred method of the present invention, reinforcement materials, such as fiber or fabric may be mixed with the concrete, or at least in the concrete used to form the top portion of the panel.

Another alternate for the improvement of the basic bridge deck panel construction process is to impress a reinforcement web fabric into the uppermost portion of the just placed concrete during the step in which concrete is placed, shored and finished, as previously described, but prior to finishing and curing.

Another alternate process to improved bridge deck panel construction is to place the concrete which is used to form the panel in multiple layers, so that a first layer of concrete placed, say up to approximately the middle of the full structural depth of the panel. Then, after the layer is properly cured, leaving the surface rough, a bonding material may be coated on the upper surface, and a second structural concrete overlay is installed to complete the full depth of the panel. This second structural concrete overlay may include a special concrete mix formulation with enhanced shrinkage and temperature characteristics, or it could include the use of fiber or fabric reinforcement in the upper portion of the

upper placement of concrete, as previously described, for control of cracking due to temperature changes.

The processes embodied by this invention wherein alternate traditional methods of constructing bridge deck panels are used, are all significantly improved by deleting two steps, and by deleting the support chairs and flexural reinforcing materials associated with those two steps from the state of the art process for constructing such panels.

The improved bridge deck panel construction process using pre-cast or prefabricated deck panels includes positioning main super-structure supporting elements and longitudinal beams, and then installing prefabricated deck panel panels, as described in alternate basic bridge deck panel construction process. The soffit forms and reinforcing are then installed, and structural concrete overlay is then placed, finished and cured, as described previously as an improvement to the basic bridge deck panel construction process described earlier. The step of placing reinforcing chairs for the upper mat and the placement of the upper reinforcing bar mat, as described in the basic process, are eliminated, as are the materials for those chairs and mats. The concrete is then placed, finished and cured, and then finally, the soffit forms are removed if necessary.

While the flexural reinforcing material most often referred to in this application is steel re-enforcing bars (re-bars), it is known that steel strands are also suitable for this purpose. Of course, flexural reinforcing material other than steel may be used in the practice of the present invention.

It is therefore seen that the present invention provides a load bearing concrete panel which is significantly less expensive to produce than existing panels, yet which meets all requirements for flexural strength imposed on such panels when used in bridging structures. This is accomplished by the removal of about one-half of the flexural reinforcing materials which are used in state-of-the-art load bearing concrete panels, and further, which is easier and less labor intensive due to the elimination of the steps which are currently necessary to place the eliminated flexural reinforcing materials. Furthermore, this is accomplished without loss of the utility of such panels, and, in fact, with the resulting panels having improved durability. In other words, by the elimination of traditionally required flexural reinforcing material from the top half of the panel, which is the principal source of panel deterioration, the present invention provides a concrete bridge deck panel structure which has sufficient flexural reinforcement to provide the appropriate amount of flexural strength, but which significantly impedes the amount and speed of deterioration of the surface of the deck panel. In preferred embodiments, a concrete bridge deck panel structure is provided in which structural flexural reinforcing material, such as steel reinforcing bars, are not required in the top half of the panel near the top surface of the panel. With the elimination of the flexural reinforcing material, such as steel reinforcing bars, a concrete bridge deck panel structure is provided in which chlorides from thawing salts and other corrosive materials do not corrode re-bars in the upper half of the concrete panel, thereby avoiding a source of significant cracking and deterioration of the top surface of the bridge deck panel. The present invention may be used in the design of concrete panels for use in new bridge construction and in rehabilitating existing bridge panel structures.

While the invention has been particularly shown, described and illustrated in detail with reference to preferred embodiments and modifications thereof, it should be understood by those skilled in art that the foregoing and other modifications are exemplary only, and that equivalent changes in form and detail may be made therein without departing from the true spirit and scope of the invention as claimed, except as precluded by the prior art.

What is claimed is:

1. A process for rehabilitating an existing concrete deck panel used as decking material in a bridge structure, said concrete deck panel being, at the time of rehabilitation, comprised of at least a deteriorated upper portion and a substantially undeteriorated concrete lower portion, each said concrete portion having a length dimension, a width dimension, having an upper surface which will come into contact with or be closely adjacent to loads which traverse the panel, said upper portion of concrete being substantially free of flexural reinforcement materials.

2. The process of claim 1 in which said over layer of concrete is constructed to resist or limit temperature change and shrinkage cracking formation at said top surface of said rehabilitated concrete panel by constructing said over layer of concrete according to practices which will resist or limit temperature change and shrinkage crack formation at said top surface of said rehabilitated panel.

3. The process of claim 2 wherein said over layer of concrete which is cast over said remaining lower portion of said existing concrete deck panel is produced by the use of a practice selected from the group consisting of the use of temperature change and shrinkage crack formation resistant concrete compositions, by including temperature change and shrinkage volume change compensating additives in concrete compositions, by utilizing concrete compositions which set to form concrete having sufficient tensile strength to resist temperature change and shrinkage cracking strain cracking, by the manner of concrete placement, by employing staged panel placement, by employing structural measures which allow temperature change and shrinkage volume change deformations to occur without restraint, by including fiber reinforcing material in said concrete compositions in at least said overlaid upper portion of said concrete in said panel in an amount sufficient to control cracking induced by temperature and shrinkage volume changes in said overlaid upper portion of said panel, and by including wire fabric reinforcing material in said concrete in said overlaid upper portion of said panel in an amount sufficient to control cracking induced by temperature change and shrinkage in said overlaid concrete upper portion of said panel.

4. The process of claim 3 in which said panel reinforcing material includes fibers in an amount and distribution sufficient to substantially resist temperature change and shrinkage cracking crack formation at the top surface of said panel.

5. The process of claim 3 in which said fibers are selected from the group consisting of metal and of polymeric material.

6. The process of claim 5 in which said fibers are metal.

7. The process of claim 5 in which said metal fibers are steel.

8. The process of claim 3 in which said panel reinforcing material includes fabric selected from the group consisting of metal wire and of polymeric material, and said fabric is present in an amount and distribution sufficient to substantially resist temperature change and shrinkage cracking crack formation at the top surface of said panel.

10. 9. The process of claim 8 in which said fabric is metal wire.

10. The process of claim 9 in which said metal wire fabric is composed of welded steel fabric located in said overlaid upper portion of said panel as a reinforcing material to restrain temperature change and shrinkage cracking at said top surface of said panel.

11. The process of claim 9 wherein said metal wire fabric is coated with water-resistant and corrosion-resistant material.

12. The process of claim 2 in which said concrete which is cast as an over layer is substantially free of materials which are readily subject to corrosion.

13. The process of claim 11 in which said panel is intended to be supported by at least a pair of separated support members.

14. The process of claim 1 in which said flexural reinforcement means in said concrete in the remaining bottom portion of said panel comprises from about 0.5% to about 8% by volume of said bottom portion of said panel.

15. The process of claim 1 in which said flexural reinforcement means in said concrete in said remaining bottom portion of said panel comprises from about at least 1% to about 4% by volume of said remaining bottom portion of said panel.

16. The process of claim 1 in which, after rehabilitation is completed, said flexural reinforcement means is disposed substantially only in the lower one-third of said rehabilitated panel.

40. 17. A method of refurbishing a deteriorated concrete panel having an upper half having an upper surface which will come into contact with or be closely adjacent to loads which traverse said panel, and a lower half having a lower surface which is spaced from loads which traverse said upper half of said panel, said concrete panel initially having flexural reinforcement means distributed throughout its structure, wherein the method includes the steps of:

removing the portion of said upper half of said panel which is deteriorated, including substantially all flexural reinforcement means in said upper half, and all portions of said lower half of said panel which has a chloride content greater than 0.1% by volume; and then

55. replacing the upper half with an over layer of concrete which is substantially free of flexural reinforcement means.

18. The process of claim 17 in which said over layer of concrete is constructed to resist or limit temperature change and shrinkage cracking formation at said top surface of said refurbished concrete panel by constructing said over layer of concrete according to practices which will resist or limit temperature change and shrinkage crack formation at said top surface of said refurbished concrete panel.

\* \* \* \* \*